

Oct. 2, 1923.

1,469,206

T. P. ANTHONY

PIPE MANUFACTURE

Filed Feb. 21, 1922

3 Sheets-Sheet 1



Inventor:  
Thomas Peacock Anthony,  
By Arthur E. Lang,  
Attorney.

Oct. 2, 1923.

1,469,206

T. P. ANTHONY

## PIPE MANUFACTURE

Filed Feb. 21, 1922

3 Sheets-Sheet 2



Thomas Peacock Notary,  
by William C. Loring,  
Attorney.

Oct. 2, 1923.

1,469,206

T. P. ANTHONY

## PIPE MANUFACTURE

Filed Feb. 21. 1922

3 Sheets-Sheet 3

### FIG. III.



Inventor:  
Thomas Peacock Taffety,  
By Arthur E. Lang Jr.  
Attorney.

Patented Oct. 2, 1923.

1,469,206

# UNITED STATES PATENT OFFICE.

THOMAS PEACOCK ANTHONY, OF EDGEWATER PARK, NEW JERSEY.

## PIPE MANUFACTURE.

Application filed February 21, 1922. Serial No. 538,238.

To all whom it may concern:

Be it known that I, THOMAS PEACOCK ANTHONY, a citizen of the United States, residing at Edgewater Park, in the county of 5 Burlington and State of New Jersey, have invented a certain new and useful Improvement in Pipe Manufacture, whereof the following is a specification, reference being had to the accompanying drawings.

10 As hereinafter described, my invention may be applied with particular advantage to pipes formed by what are known as centrifugal processes. In such processes, a cylindrical mold is rotated while molten iron 15 is poured therein so that the so-called centrifugal force which rotation develops in a revolving mass, compels the molten iron to line itself in a shell of uniform thickness on the inside of the rotating mold. Ordinarily, such molds are water cooled upon their 20 exterior, with the result that the iron cast therein is chilled upon its outer surface to a depth of approximately one thirty-second of an inch; necessitating a subsequent annealing process to soften the surface of the 25 pipe which is thus hardened. Moreover, pipe thus cast is of much denser composition and far more resistant to stresses than pipe cast in ordinary sand molds, but is 30 more rapidly corroded by moisture; the difference in that respect being probably due to the characteristic change in the composition of the metal of the pipe which is incident to the centrifugal method of casting 35 the same; for instance, metal from the same heat cast centrifugally and in ordinary sand molds shows upon analysis the following differences in proportions of five of the ingredients thereof:

fore, it is to be noted that the hardness of the outer surface of such castings is due to the fact that the quicker solidification and further cooling of the metal coming in contact with the cooled molds aforesaid causes the retention of much combined carbon and thus prevents the formation of graphite in the portions of the casting thus chilled. The purpose and effect of the annealing 60 65 herein contemplated is to convert the hard brittle cementite into particles of soft graphitic carbon and, incidentally to eliminate some of the carbon in combination with such oxygen as may reach it. However, the 70 principal object and effect of the process herein contemplated is the graphitizing of the cementite at a temperature above the critical point  $Ac_{3,2,1}$  of the cast iron and, of course, below its temperature of solidifica- 75

As hereinafter described such effect is attained by controlling the rate of cooling of the centrifugally cast pipe from its solidification point until it is annealed; and preferably in a confined atmosphere in an annealing oven, to which said pipes are withdrawn from their respective molds, while at a temperature above 1000° F.

As hereinafter described, the annealing 80 85 process above contemplated is preferably effected by removing each centrifugally cast pipe from its mold, axially, into the confined annealing atmosphere and rotating said pipe upon its axis while progressing the 90 latter transversely with respect to its original position, into regions of successively lower temperature in said confined atmosphere until said pipe has cooled to less than 500° F.; and then withdrawing said pipe 95 from said secluded atmosphere into the open atmosphere.

As hereinafter described, I find it convenient to employ an annealing oven having guide rollers to receive and support the pipe 100 shifted axially into said oven, and a series of rollers, mounted to rotate upon axes parallel with the axis of said pipe and arranged to successively engage said pipe and rotate it upon its axis while progressing the latter 105 transversely with respect to its original position. Such an oven is conveniently provided with a source of heat whereby its temperature may be controlled and such that it may be maintained at the proper high temperature at the region of introduction of said pipe.

|         | Centrifugal. | Sand.     |
|---------|--------------|-----------|
|         | Per cent.    | Per cent. |
| C.....  | 3.45         | 3.67      |
| Mn..... | .49          | .61       |
| S.....  | .053         | .044      |
| P.....  | .563         | .654      |
| Si..... | 2.48         | 2.00      |

Therefore, the unquestionable advantages of centrifugal cast iron pipe as compared with sand molded pipe with respect to the strength and initial cost thereof are offset by the necessity for annealing the centrifugal cast pipe.

Therefore, it is an object and effect of my invention to minimize the cost of the required annealing, as far as possible. There-

My invention includes the various novel features of construction and arrangement hereinafter more definitely specified. The rotary mold and its appurtenances herein disclosed are claimed in my copending application Serial No. 507,824, filed October 15, 1921, for Letters Patent of the United States.

Fig. I is a diagrammatic side elevation of a casting and annealing apparatus which may be conveniently used in accordance with my invention.

Fig. II is a diagrammatic vertical sectional view of the rotary mold and its appurtenances indicated in Fig. I.

Fig. III is a diagrammatic vertical sectional view of an annealing oven adapted to receive pipe removed axially from the apparatus shown in Fig. I, and including means for rotating such a pipe upon its axis while shifting the latter transversely, to the region of discharge from said oven.

In said figures; the pipe 1 is being formed by molten metal 2 poured through the spout 3 from the ladle 5 which is tiltable upon the pivot 6 at the outer end of said spout. Said pipe 1 is formed within the rotary mold comprising the inner shell 8 surrounded by insulating material 9 within the outer casing 10. Said casing 10 is provided with annular tracks 11 and 12 whereby said mold may be supported for rotation upon suitable rollers 13. Said mold may be rotated by a belt 14 encircling the belt flange 15, while the entire mold is axially shifted with respect to said spout 3, which may remain stationary. The exterior of said mold may be chilled by water sprayed thereon from the pipe 17 within the water shield 18. The dry comminuted lining material 20 may be sprayed within the said pipe 1 through the nozzle 21 of the conduit 22 which may be held stationary with said spout 3 while the application of the molten metal 2 and said lining material 21 in a helical path is determined by the relative axial movement of said pipe 1 with respect to said spout 3 and conduit 22. Rotation of said mold may be conveniently effected by an electric motor 25 mounted upon a suitable carriage 26, provided with four supporting rollers 27 upon tracks 28 parallel with the axis of rotation of said pipe 1; while axial movement of said carriage 26, and said pipe 1 rotating therein, may be effected by a hydraulic cylinder 30 engaging a plunger 31 attached to said carriage.

I find it desirable to omit the vitreous lining from the bell end 34 of said pipe 1 as indicated in Fig. II; for the reason that said bell end is used to retain molten lead poured therein to form a joint with the opposite end of a similar pipe, and such a joint is preferably made with the lead in direct contact with the iron. Therefore, I have shown in Fig. II the mold tube 35 arranged to hold

a core of insulating material 36 in such position as to cover the inner surface of said pipe 1 at its bell portion 34 and thus prevent the deposit of vitreous coating material 20 thereat.

The principal ingredient of the vitreous coating material aforesaid may be glass cullet comminuted to a fineness varying from that of powdered sugar to granulated sugar. Although a temperature in excess of 2000° F. may be required to fuse glass alone and in bulk; it fuses at a much lower temperature when thus comminuted and mixed with other ingredients to form such vitreous coatings as are employed for lining cooking utensils. Such compositions are fusible throughout a range of 900° to 1500° F. and are satisfactory for use as above described. I have found it convenient to spray such material upon the interior of the pipe 1 by means of compressed air at eighty pounds per square inch, because I have had such spraying means at hand. However, such comminuted lining material may be otherwise applied. For instance, it may be delivered through a perforated vibratory distributor, without an air blast. Moreover, as the specific gravity of such lining material is approximately 2.5; it may be deposited upon the inflowing stream of molten iron and distributed by the latter; the centrifugal effect aforesaid forcing the molten metal outward and leaving the lining material at the inner surface of the pipe 1. The latter method of application has the advantage that it insures a deeper penetration of the vitreous material with respect to the pores of the metal at the inner surface of the pipe thus coated.

I have found it convenient to rotate such centrifugal apparatus as indicated in Figs. I and II at the rate of 550 revolutions per minute and to effect the relative axial movement of the spout 3 and mold 8 at the rate of approximately two feet per minute.

When a pipe of the desired thickness is thus centrifugally cast in said mold and preferably while it is at a temperature above 1000° F.; it is removed from said mold, axially, into the confined atmosphere 39 within the oven 40. Such removal may be effected by engaging the bell end of said pipe when it is presented by the casting apparatus in the position nearest to said oven and permitting the mold to be retracted by the hydraulic means above described while said pipe is shifted axially forward into said oven. To facilitate the introduction of said pipe 1 to said oven 40; the latter is provided with a series of rollers 41 mounted to rotate upon axes 42 at right angles to the axis of said pipe 1. Said pipe 1 is then rotated upon its axis to remove it from said rollers onto a series of rollers 43 which are mounted to rotate upon axes coincident with shafts 44 parallel with the axis of said pipe 1.

Said rollers 43 are connected by gears 46 and turned by any suitable means, for instance, by a motor 47 having a shaft 48 provided with a worm 49 engaging the worm wheel 50 upon the initial end shaft 44. Each of said rollers 43 has a recessed portion 52 and they are rotated in the direction of the arrows marked thereon in Fig. III so as to progress said pipe 1 transversely with respect to its original position into regions of successively lower temperature in said confined atmosphere 39, until said pipe has cooled to less than 500° F. and is annealed. Said pipe may then be withdrawn from the secluded atmosphere 39, through the opening 60 in said oven 40 into the open atmosphere.

I find it convenient to provide said oven 40 with an oil or gas burner 62 whereby said confined atmosphere 39 may be maintained at a temperature above 1000° F.; and preferably above 1400° F., at the region of introduction of said pipe 1. The products of combustion from said burner 62 pass downwardly to the flue 64 through which they escape to the outer atmosphere.

It may be observed that the construction and arrangement above described are such that said atmosphere 39 is hottest at the region of introduction of said pipe and the temperature thereof decreases toward the right hand end of the oven, as shown in Fig. III, and the general construction and arrangement above described are such as to enable the operator to control the rate of cooling said pipe 1 from its solidification point until it is annealed.

It may be observed that said pipe 1 may be annealed to what is termed "black heart" condition without any oxidizing means, in much less time and from a lower temperature, than is required for producing what is known as the "white heart" condition thereof. However, said burner 62 may be constructed and arranged to produce an oxidizing flame, if it is desired that said pipe 1 shall be annealed to the "white heart" condition. In either case, it is essential that the temperature of said pipe shall be controlled and gradually reduced from above the critical  $Ac_{321}$  point of the metal of which they are cast; in order to graphitize the carbon at the outer surface of said pipe which otherwise would form hard brittle cementite. It may be observed that the "white heart" condition of cast iron above contemplated is characterized by coarse fracture and structure of the metal, because of the high and prolonged heating to which it is exposed; so that castings in that condition are slightly weaker than when in the "black heart" condition.

It may also be observed that the presence of sulphur and manganese in the cast iron promotes the retention of combined carbon as hard cementite, whereas, the presence of

silicon and of large percentages of total carbon facilitate the process of annealing or malleabilizing above contemplated.

Although I have found the apparatus above described convenient for the purpose set forth; I do not desire to limit myself to the specific construction and arrangement thereof, as it is obvious that various modifications may be made therein without departing from the essential features of my invention, as defined in the appended claims. For instance; the confined atmosphere to which the pipes are subjected during their annealing above contemplated may include any element adapted to facilitate the desired softening of their outer surfaces. Such material may be directed to the pipe 1 from the conduit 65 shown in Fig. III; or, the pipe 1 may be temporarily encased in a container 67 with any decarbonizing material, for instance, powdered iron ore 68 or other oxides. Or such a container 69 may hold inert refractory material 70, such as sand or clay, or diatomous earth, around the pipe 1 until the latter cools to the desired degree. Of course, the pipe 1 may be merely imbedded in suitable refractory material 70, during its cooling, without any annealing oven; the essential thing being that the heat in the pipe when it is cast shall not be permitted to escape until the metal is annealed.

I claim:

1. The process of making cast iron pipe, which consists in removing said cast pipe from the mold, axially, into a confined atmosphere maintained at a temperature above 1400° F. at the region of introduction of said pipe; and while said pipe is at a temperature above 1000° F.; rotating said pipe upon its axis while progressing the latter transversely with respect to its original position, into regions of successively lower temperature in said confined atmosphere, until said pipe has cooled to less than 500° F.; and then withdrawing said pipe from said secluded atmosphere into the open atmosphere.

2. The process of making cast iron pipe, which consists in removing said cast pipe from the mold, into a confined atmosphere maintained at a temperature above 1400° F. at the region of introduction of said pipe; and while said pipe is at a temperature above 1000° F.; rotating said pipe upon its axis while progressing the latter transversely with respect to its original position, into regions of successively lower temperature in said confined atmosphere, until said pipe has cooled to less than 500° F.; and then withdrawing said pipe from said secluded atmosphere.

3. The process of making cast iron pipe, which consists in removing said cast pipe from the mold, into a confined atmosphere

5 maintained at a temperature above 1000° F. at the region of introduction of said pipe; and while said pipe is at a temperature above 1000° F.; rotating said pipe upon its axis while progressing the latter transversely with respect to its original position, into regions of successively lower temperature in said confined atmosphere, until said pipe has cooled to less than 500° F.; and 10 then withdrawing said pipe from said secluded atmosphere.

4. The process of making cast iron pipe, which consists in removing said cast pipe from the mold, into a confined atmosphere 15 maintained at a temperature above 1000° F. at the region of introduction of said pipe; and while said pipe is at a temperature above 1000° F.; progressing the pipe transversely with respect to its original position, into 20 regions of successively lower temperature in said confined atmosphere, until said pipe has cooled to less than 500° F.; and then withdrawing said pipe from said secluded atmosphere.

25 5. The process of making cast iron pipe, which consists in removing said cast pipe from the mold, into a confined atmosphere maintained at a temperature above 1000° F. at the region of introduction of said pipe; 30 and while said pipe is at a temperature above 1000° F.; progressing the pipe into regions of successively lower temperature in said confined atmosphere, until said pipe has cooled to less than 500° F.; and then 35 withdrawing said pipe from said secluded atmosphere.

6. The process of making cast iron pipe, which consists in removing said cast pipe from the mold, into a confined atmosphere 40 and while said pipe is at a temperature above its critical point  $Ac_{3.2.1}$ ; progressing the pipe into regions of successively lower temperature in said confined atmosphere, until it has cooled below said point; and 45 then withdrawing said pipe from said secluded atmosphere.

7. The process of making cast iron pipe, which consists in removing said cast pipe from the mold, into a confined atmosphere, 50 and while said pipe is at a temperature above its critical point  $Ac_{3.2.1}$ ; and retaining said pipe in said confined atmosphere until it is annealed.

8. The process of making cast iron pipe, 55 which consists in removing said pipe from the mold, into a confined atmosphere and while said pipe is at a temperature above 1000° F.; and retaining said pipe in said atmosphere until it is annealed.

60 9. The process of making cast iron pipe, which consists in rotating and controlling

the rate of cooling of said pipe from its solidification point until it is annealed; by retarding the loss of the initial heat of fusion of said metal.

10. The process of making cast iron pipe, which consists in rotating a mold while pouring molten metal therein, until a pipe of the desired thickness is thus centrifugally cast in said mold; in contact with a rigid matrix in said mold, contemporaneously applying a vitreous lining material to the interior of said pipe, in a dry comminuted state, and thus forming a vitreous lining in said pipe; removing said cast pipe from said mold, into a confined atmosphere and while said pipe is at a temperature above its critical point; and retaining said pipe in said confined atmosphere until it is annealed.

80 11. The process of forming a cast iron pipe with a vitreous lining, of less specific gravity than iron, which consists in delivering both molten iron and the lining material to the interior of a mold, with said lining material in a comminuted state, at a temperature below its fusing point, while rotating said mold at such speed as to centrifugally distribute both said metal and lining material in said mold, until a pipe of the desired thickness is thus centrifugally cast in said mold, in contact with a rigid matrix in said mold; the inner surface of said pipe being at such temperature as to fuse the lining material; removing said cast pipe from said mold, into a confined atmosphere; and retaining said pipe in said confined atmosphere until it is annealed.

85 12. The process of forming a cast iron pipe with a vitreous lining, of less specific 100 gravity than iron, which consists in delivering both molten iron and the lining material to the interior of a mold, with said lining material in a comminuted state, at a temperature below its fusing point, while 105 rotating said mold at such speed as to centrifugally distribute both said metal and lining material in said mold, until a pipe of the desired thickness is thus centrifugally cast in said mold, in contact with a rigid 110 matrix in said mold; the inner surface of said pipe being at such temperature as to fuse the lining material; and controlling the rate of cooling of said pipe from its solidification point until it is annealed.

115 In testimony whereof, I have hereunto signed my name at Burlington, New Jersey, this 18th day of February, 1922.

THOMAS PEACOCK ANTHONY.

Witnesses:

EVA T. AARONSON,  
A. W. DRESSER.